# EUROPEAN PATENT APPLICATION

(11) **EP 0 099 618 A2**
(43) Date of publication of application: **01.02.1984**
(21) Application number: 83302010.0
(22) Date of filing: 11.04.1983
(51) Int. Cl.: C21D 8/12, H01F 1/16

(54) **Method for producing cube-on-edge oriented silicon steel**

(30) Priority: 19.07.1982 US 399937
(71) Applicant: ALLEGHENY LUDLUM STEEL CORPORATION, Pittsburgh Pennsylvania 15222 (US)
(72) Inventor: Miller, Robert Frederick, Evans City Pennsylvania 16033 (US)
(74) Representative: Sheader, Brian N.

(57) **Abstract**

An improvement in the manufacture of cube-on-edge oriented silicon steel; the improvement comprises serrating said steel either before or after final texture annealing, whereby reduced watt loss is achieved.

## Description

This invention relates to a method of producing cube-on-edge oriented silicon steel.

Cube-on-edge oriented silicon steel in the form of sheets is known for use in various electrical applications including transformer cores. With cube-on-edge silicon steel the alloy is characterized by secondary recrystallization in the (110) (001) position which is termed the cube-on-edge position. This material in sheet form has the direction of easy magnetization in the direction of rolling. In applications for this material, and specifically when used in the manufacture of transformer cores, the material is required to have reduced watt loss, because the consumption of electrical energy decreases as iron loss decreases.

It is accordingly an object of the present invention to provide a method whereby in the manufacture of cube-on-edge silicon steel reduced watt loss may be achieved.

The present invention provides a method of producing cube-on-edge silicon steel, characterized by reduced watt loss, including the steps of hot-rolling, cold-rolling with intermediate annealing and a final texture annealing, comprising serrating said steel after texture annealing.

In the practice of the invention cube-on-edge silicon steel to which the invention is directed is conventionally processed by hot rolling and cold rolling with intermediate annealing. Thereafter, the steel is subject to texture annealing to produce the desired secondary recrystallization in the (110) (001) position. It has been found, in accordance with the present invention, that either prior to this final texture annealing or after final texture annealing the watt loss of the steel may be reduced by serrating the steel, with the serrating preferably being in a direction essentially perpendicular to the (001) crystal direction. The depths of the serrations are typically 0.025mm (001"), but may be within the range of .05 to .005mm (.002" to .0002"), the widths of the serrations are typically .lmm (.004") but may be within the range of .25 to .0025mm (.010" to .0001"), and the intervals or distance from serration to serration may be within the range of 5 to 12.7mm (.2 to .5"). Although the practice of the invention is applicable to cube-on-edge silicon steel generally it is particularly suited to the following compositions in percent by weight:

By way of specific example, five 12-strip Epstein packs of 10.2 mil (.259mm) final normalized SX-14 silicon steel composition were provided for testing. Two of the final normalized packs were used as control specimens (control 1 and control 2) and the remaining three were scribed essentially perpendicular to the rolling direction and the (001) crystal direction to provide serrations in accordance with the practice of the invention. The interval between serrations was varied between lOmm and 5mm. All specimens were coated with a water slurry of 300 cc of water, 46gm. of MgO and 2gms. of H₃BO₃ and annealed in hydrogen for 12 hours at a temperature of 2150°F (1177°C). After annealing, the resulting magnetic properties were determined.

^{*}Numbers in parentheses are in SI units viz. webers per ampere turn meter.

As may be seen from the above data the samples which were serrated exhibited reduced watt loss over the control samples.

Single strip tests were made on eight strips from each aforementioned pack to determine if tension would further reduce the watt loss of the serrated strips. After testing under tension the eight strips from each pack were stress coated by applying a commercial tension-producing coreplate and retested for watt loss. The average watt loss for the eight single strips is as follows.

### Heat 154684-lA

As may be seen from this data stressing in combination with serrating provided a further improvement with respect to reducing watt loss over serrating alone.

One 20-strip Epstein pack (Heat 156625-3 Out) which had been texture annealed with a conventional MgO + .75 B coating was serrated with a metal scribe at intervals of 7.5mm perpendicular to the rolling direction. Strips were stress relieved at 1177⁰C (2150°F) for eight hours in hydrogen following the application of the scribe lines. The following magnetic properties were determined:

Before
Scribing 1940 (2.44x10⁻³) 13,440(1.70x10⁻³) .651 (1.44) After
Scribing 1919 (2.41x10⁻³) 16,300(2.05x10⁻³) .609 (1.34)

As may be seen from the above the practice of the invention is effective when serrating is performed either before or after the final texture annealing.

## Claims

1. A method of producing cube-on-edge silicon steel, characterized by reduced watt loss, including the steps of hot-rolling, cold-rolling with intermediate annealing and a final texture annealing, characterized in comprising serrating said steel after texture annealing.

2. A method according to claim 1,characterized in that said steel is serrated in a direction essentially perpendicular to the (001) crystal direction.

3. A method according to claim 1 or 2, characterized in that serrating is performed to provide serrations having a depth of .05 to .005mm (.002 to .0002 in.), a width of .25 to .0025mm (.010 to .0001 in.) and said serrations are at intervals within the range of 5 to 12.7mm (.2 to .5 in.).

4. A method according to claim 1, 2 or 3, characterized in stressing said steel to further reduce the watt loss.
